

## UNITED STATES PATENT OFFICE

2,177,448

WOOD TREATING AND PRESERVING  
COMPOSITIONHoward B. Carpenter, Elizabeth, N. J., assignor  
to Penola, Inc.No Drawing. Application October 8, 1935,  
Serial No. 44,057

6 Claims. (Cl. 134—78.6)

This invention relates to improved coal tar compositions, and more particularly to compositions containing coal tar dissolved in selected fractions of petroleum oil and suitable for the treatment and preservation of wood.

It is common practice to use creosote, a distillate fraction of tar, for wood impregnation. Coal tar and the heavier residual fractions thereof have also been suggested for this use but are generally considered less desirable than creosote on account of their higher viscosity and lower toxicity. Attempts to reduce the viscosity of coal tar by dilution with ordinary petroleum oil fractions are generally unsuccessful, due to the low solubility of coal tar in these oils.

It has now been discovered that coal tar is readily soluble in petroleum oils having an aniline point below about 50° F. and that coal tar compositions containing such oils are highly effective for the treatment and preservation of wood. Oil fractions of suitable viscosity and/or volatility are selected for the particular use of the coal tar composition derived. Volatile oils may be used as solvents for coal tar in the preparation of surface coating compositions, such as coal tar paints and varnishes. For example, petroleum oils of such low aniline points and boiling below about 400 to 450° F. are suitable, and oils of even higher boiling range may be used. Higher boiling oils, boiling generally above 400° F., are used in the preparation of coal tar compositions to be used for the impregnation of wood.

In preparing wood preservatives suitable for use as a creosote substitute for impregnating wood, the petroleum oils used should have a flash point above about 150° F., and preferably above about 200° F., and an aniline point below about 50° F., and preferably below about 20° F. The oils should also have a sufficiently low viscosity so that the viscosity of the resulting blend with coal tar is suitable for wood impregnation, for example, about 25 to 45 seconds Saybolt at 210° F. This is given merely as an illustration of a suitable range, as wide variations in the viscosity of the treating medium are permissible in wood impregnation, and can be offset by suitable variations in treating pressures and temperatures. Viscosities of about 30 to 40 are preferred. Such petroleum oil fractions may be obtained by subjecting petroleum oils to distillation, extraction, cracking, or destructive hydrogenation or to any suitable combination of these treatments. The oils used are preferably from a largely aromatic

or naphthenic source, such as the California and asphalt-base crudes.

A suitable method of preparing oil fractions for the present invention is to separate from a petroleum oil or fraction thereof the aromatic, naphthenic and olefinic compounds by means of a selective solvent, such as furfural, phenol or liquid sulfur dioxide. The extract may then be distilled to secure a distillate fraction of suitable boiling range and viscosity for the purpose desired or the initial petroleum fraction may be subjected to a similar treatment before extraction. Suitable oils for the present invention may also be obtained by subjecting petroleum oils and fractions thereof to destructive hydrogenation under conditions favoring the formation of aromatic hydrocarbons.

It is known that petroleum distillates may be hydroformed by destructive hydrogenation at elevated temperatures and pressures to produce products essentially different from those produced by simple hydrogenation or even by destructive hydrogenation at lower temperatures. For example, the hydroformed products when used as motor fuels possess anti-knocking characteristics to a much greater degree than shown by the original oils or by products of other types of hydrogenation. These hydroformed products are produced from petroleum distillates such as burning oil and gas oil and in general from petroleum oils of a boiling range including that of gasoline and extending up to about 650 to 700° F. or somewhat higher. These distillate oils are passed in vapor phase with free hydrogen over suitable catalysts at a pressure in excess of 20 atmospheres and preferably 50 to 200 atmospheres or higher and at a temperature above about 900° F. and preferably within the range of about 930 to 1050° F. with a suitable partial pressure of hydrogen and time of contact to secure a destructive hydrogenation without the formation of appreciable amounts of polymerized or coky material. The hydrogen supplied is preferably within the range of about 1000 to 4000 cubic feet per barrel of feed oil, the amount generally depending upon the gravity and boiling range of the charging stock. A greater proportion of hydrogen may be used with suitable variation in feed rate, temperature and pressure as is known in the art. The feed rate depends upon the reaction temperature, and other operating conditions such as the partial pressure of hydrogen and may be suitably about 1.5 to 4 volumes of oil per volume of catalyst filled reaction space per hour. The catalysts preferably com-

prise the oxides or sulfides of the metals of group VI of the periodic table with suitable promoters of the alkaline earth or earth oxides. Such catalysts are insensitive to sulfur poisoning and are suitably classified as sulfactive.

This destructive hydrogenation process is conveniently described as a "hydroforming" process and the liquid products thereof are identified as "hydroformed" products for the purpose of this invention and the claims.

A preferred oil for use according to the present invention is obtained by hydroforming extracts obtained by treating petroleum oils with selective solvents, such as liquid sulfur dioxide.

The following examples are presented to illustrate a preferred modification of this invention, but are not intended in any way to constitute a limitation thereof.

*Example 1*

The extract obtained on treating a kerosene distillate fraction of a naphthenic crude oil with liquid sulfur dioxide is heated to remove 40% of the more volatile components as distillate. The residue, constituting 60% of the sulfur dioxide extract, is subjected to destructive hydrogenation at a temperature between 930 and 1050° F., and a pressure of 3000 lbs. per square inch in the presence of catalysts containing oxides and/or sulfides of metals of group VI. The resulting hydro-formed liquid product is distilled to recover as distillate fractions boiling below about 410° F.

Forty parts by volume of the residual fraction are mixed with sixty parts of a tar consisting of the non-aqueous portion of the liquid distillate obtained by the carbonization of bituminous coal. The resulting mixture is a substantially homogeneous liquid and shows at most only a trace (less than 1%) of insoluble material.

The characteristics of the hydroformed oil, the coal tar and the resulting mixture are given in the following table:

| 45                                | Distillation* | Oil           | Coal Tar | Mixture |
|-----------------------------------|---------------|---------------|----------|---------|
| Below 410° F.                     | 0.0           | 5.8           | 2.4      |         |
| 410 to 455                        | 12.0          | 12.0          | 12.3     |         |
| 455 to 518                        | 68.0          | 5.7           | 24.2     |         |
| 518 to 599                        | 19.4          | 10.1          | 19.1     |         |
| 599 to 671                        | Trace         | 13.8          | 10.2     |         |
| Residue                           | Trace         | 52.6          | 31.8     |         |
| Aniline point °F.                 | -70           |               |          | 37      |
| Viscosity, sec. Saybolt @ 210° F. | 31            | 125 (approx.) |          |         |

\*Standard Distillation of Creosote, #11e, Manual of Recommended Practice of American Wood-Preservers' Association.

If an ordinary cracked petroleum oil fraction of similar boiling range is substituted for the hydroformed oil in the above example, the resulting mixture of oil and coal tar is completely coagulated into a semi-solid gel, which is wholly unsuitable for use as a wood impregnant.

In addition to serving as a solvent and diluent for the coal tar, the petroleum oil fraction used in the above example also has exceptionally good

preservative qualities. Its toxicity is 0.03%, which compares favorably with an average toxicity of about 0.05% for creosote and 0.2% to 0.4% for coal tars. This toxicity, determined by the standard method used by wood preservers, is the concentration of the oil in malt-agar media necessary to completely inhibit growth of a test fungus, *Fomes annosus*.

The aniline point of the petroleum oil fraction used in the above example is -70° F. Such aniline points below the freezing point of aniline are determined by mixing the oil to be tested with an oil of known high aniline point and calculating from the aniline point of the mixture, the aniline point of the added oil. Petroleum oils having higher aniline points of 20 and even 50° F. and of suitable viscosity, volatility and flash for the wood preservative or treating purposes desired may be substituted in the above example for the oil used therein. While coal tars are often somewhat less soluble in these oils of higher aniline point, the mixtures nevertheless are fluid and are far more suitable for wood treating than are mixtures of coal tar with ordinary petroleum oils.

This invention is not to be limited by any theoretical explanations or examples which have been presented herein solely for purpose of illustration, but is limited only in the following claims, in which it is desired to claim all novelty in so far as the prior art permits.

I claim:

1. An improved wood preservative composition comprising a solution of coal tar in a petroleum oil fraction which will not reduce the fungicidal properties of the tar and which has an aniline point below about 50° F., said oil being obtained by "hydroforming" an extract of a petroleum oil having a substantial amount of naphthenic hydrocarbons and which is separated from said petroleum oil by means of a selective solvent.

2. An improved wood preservative composition comprising a solution of coal tar in a petroleum oil fraction which will not reduce the fungicidal properties of the tar and which has an aniline point below about 50° F., said oil being obtained by "hydroforming" a sulfur dioxide extract of a petroleum distillate oil fraction.

3. An improved wood preservative composition comprising a solution of a coal tar in a solvent which will not reduce the fungicidal properties of the tar, consisting of a hydroformed sulfur dioxide extract of a petroleum distillate oil fraction, said solvent having an aniline point below about 50° F. and a flash point above about 150° F.

4. Composition according to claim 3, in which said solvent has an aniline point below about 20° F.

5. Composition according to claim 3, in which said solvent has an aniline point of about 20 to -80° F. and a flash point above about 200° F.

6. Composition according to claim 3, having a viscosity of about 30 to 40 seconds Saybolt at 210° F.

HOWARD B. CARPENTER.

65